

## UNITED STATES PATENT OFFICE

2,639,985

## BEARING AND STEEL THEREFOR

**Karl F. Schauwecker, Franklin Park, Ill., assignor to United States Steel Corporation, a corporation of New Jersey**

No Drawing. Continuation of application Serial No. 109,803, August 11, 1949. This application April 30, 1951, Serial No. 223,830

2 Claims. (Cl. 75—124)

1

This invention relates to improvements in bearings and steels therefor.

The service life of bearings, such as ball and roller bearings, is in many installations to a large degree dependent on the resistance thereof to softening under the high temperatures to which they are subjected. Moreover in forming bearings, it is necessary that the steel have a high degree of forgeability.

It is accordingly an object of the present invention to provide steel bearings which have an increased service life despite their being subjected to high temperatures.

It is a further object to provide steels for bearings which are relatively stable at high temperatures and which have a high degree of resistance to softening at elevated temperatures.

It is another object to provide steels for bearings which will regain to a large degree any hardness loss due to being subjected to unduly high temperatures in service.

It is a further object to provide such qualities in a steel which is highly forgeable.

I have discovered that the foregoing objects can be attained by alloying between .75 and 1.25% aluminum and .20 and .55% silicon, with the aluminum plus silicon content being between 1.00 and 1.75%, with hardenable bearing steel. While this is beneficial to hypereutectoid bearing steels generally, it is particularly true of hypereutectoid bearing steels having a room temperature Rockwell C hardness of at least 60 after quenching. Preferably the bearing steels of this invention will contain between .95 and 1.15% carbon, .25 to .50% manganese, .20 to .50% silicon, .35% maximum nickel, 1.35 to 1.65% chromium, .35% maximum copper with the balance iron except for residual elements in common amounts.

The hereinafter presented data obtained from the heats of steels shown in Table I produced by conventional practice in a high-frequency induction furnace are believed to clearly illustrate ability of my improved steel to harden and retain its hardness despite being subjected to high temperatures.

2

TABLE I

|   | Heat No. | C    | Mn  | Si  | Ni   | Cr   | Mo  | Al   |
|---|----------|------|-----|-----|------|------|-----|------|
| 5 | 1        | 1.02 | .59 | .50 | —    | 1.50 | —   | None |
|   | 2        | 1.09 | .62 | .59 | .21  | 1.58 | .24 | 1.18 |
|   | 3        | 1.02 | .35 | .29 | .21  | 1.51 | .24 | None |
|   | 4        | 1.10 | .41 | .30 | —    | 1.44 | —   | 1.12 |
|   | 5        | .64  | .98 | .20 | —    | —    | .24 | None |
|   | 6        | .63  | .99 | .41 | —    | —    | .25 | 1.05 |
|   | 7        | .51  | .75 | .21 | 1.75 | .99  | .25 | None |
|   | 8        | .52  | .80 | .23 | 1.65 | .80  | .26 | 1.06 |

The hardness of certain of the foregoing steels was determined after heating for 20 minutes at the temperatures set forth in Table II. The specimens used were about 1 inch in cross section and the hardness measured with a diamond penetrator. For the sake of convenience of comparison, the values obtained were converted to Rockwell C readings, using conversion figures recommended by the American Society for Testing Materials (E-48-437).

TABLE II

|    | Testing to—             | 3—No Al | 4—Al | 7—No Al | 8—Al |
|----|-------------------------|---------|------|---------|------|
| 25 | Room (before test)..... | 66.0    | 65.5 | 63.0    | 62.0 |
|    | 200° F.....             | 65.5    | 66.0 | 62.0    | 58.0 |
|    | 300° F.....             | 61.5    | 65.5 | 59.0    | 58.0 |
|    | 400° F.....             | 53.0    | 60.5 | 54.0    | 55.0 |
|    | 500° F.....             | 55.0    | 57.5 | 49.0    | 52.0 |
|    | 600° F.....             | 43.0    | 55.0 | 45.0    | 50.0 |
|    | Room (after test).....  | 56.0    | 63.0 | 45.0    | 54.0 |

An examination of this table shows that the decrease of hardness of specimens heated to elevated temperatures is much slower for the steel containing 1% aluminum and the recovery after return to room temperature much greater. It is also noted that these qualities are much more pronounced in the hypereutectoid steel containing aluminum and low nickel.

The resistance to softening of the steels of my invention upon holding at elevated temperatures for prolonged periods of time is illustrated in the following Table III. This table gives the room temperature hardness values in Rockwell C figures obtained after heating, for the temperatures and times indicated, specimens quenched in water from above the  $A_{e1}$  point and preferably above 1475° F.

3  
TABLE III

|                       | 1-No Al | 2-Al | 5-No Al | 6-Al | 8-Al |
|-----------------------|---------|------|---------|------|------|
| As quenched           | 65.0    | 66.0 | 64.5    | 62.0 | 64.0 |
| Drawn at 350° F. for: |         |      |         |      |      |
| 2 Hours               | 60.3    | 62.2 | 58.0    | 57.5 | 55.0 |
| 4 Hours               | 60.6    | 62.8 | 56.0    | 55.0 | 54.5 |
| 28 Hours              | 60.8    | 62.8 | 58.0    | 58.0 | 52.0 |
| Drawn at 450° F. for: |         |      |         |      |      |
| 2 Hours               | 60.4    | 62.3 | 54.0    | 58.0 | 55.0 |
| 4 Hours               | 60.6    | 62.8 | 52.0    | 58.0 | 56.0 |
| 28 Hours              | 58.2    | 62.8 | 55.5    | 55.0 | 53.0 |
| Drawn at 550° F. for: |         |      |         |      |      |
| 2 Hours               | 59.4    | 62.1 | 55.0    | 56.0 | 53.0 |
| 4 Hours               | 59.4    | 62.2 | 54.0    | 57.0 | 54.0 |
| 28 Hours              | 59.2    | 62.1 | 52.0    | 56.6 | 51.0 |

The figures of the foregoing Table III show the influence of 1% aluminum in resistance to softening after various periods at various temperatures. The difference is again much more pronounced in the hypereutectoid steels.

It is clear from the tables that alloying hardenable steels with about 1% of aluminum renders them more resistant to the softening effect of heating. This permits operation of bearing made therefrom at high temperatures, and greatly reduces the dangers caused by softening of steel induced by temporary overheating. In the case of heat No. 4, for example, no damage for bearings composed of such steel can be expected after overheating for 20 minutes at 600° F., while the same overheating would seriously affect bearings of the same composition without aluminum.

containing about 1½% aluminum plus silicon developed satisfactory as quenched hardness, but that the steel with more than 1.75% aluminum plus silicon did not give satisfactory hardness. Moreover, after drawing at 550° F. for 28 hours, the steel containing less than 1% aluminum plus silicon did not retain hardness for satisfactory service at such temperature, falling below 60 R<sub>c</sub>. The steel with over 1.75% aluminum plus silicon retained its hardness, but was not sufficiently hard as quenched. It should be noted that the 1½% aluminum plus silicon not only developed satisfactory hardness but also retained its hardness satisfactorily for bearing service.

The following Table VI indicates the results of upset forging tests made on specimens ½" diameter x 1" specimens of the above strips which were reduced to ⅛" and ¼" thickness.

TABLE VI  
Forgeability

| Heat No. | Upset Forgings<br>Units ½"<br>dia. x 1" | Forging Temperature, ° F.           |                           |                            |                             |
|----------|-----------------------------------------|-------------------------------------|---------------------------|----------------------------|-----------------------------|
|          |                                         | 1,850                               | 1,950                     | 2,050                      | 2,150                       |
| 9        | 1/8                                     | Surface O. K.<br>do<br>do           | Surface O. K.<br>do<br>do | Surface O. K.<br>do<br>do  | Surface O. K.<br>Do.<br>Do. |
| 10       | 1/8                                     | do                                  | do                        | do                         | do                          |
| 11       | 1/8                                     | Unforgeable<br>Ruptured<br>Ruptured | Ruptured<br>Surface O. K. | Ruptured<br>Surface Rough. | Surface Rough.<br>Ruptured  |

Such beneficial qualities, however, are only obtainable when the aluminum plus the silicon content is maintained in the range of 1.00 to 1.75%. To further illustrate this, the following heats of steel were made and tested as follows:

TABLE IV

| Heat No. | C       | Mn      | Si      | Cr      | Al      | Al+Si   |
|----------|---------|---------|---------|---------|---------|---------|
|          | Percent | Percent | Percent | Percent | Percent | Percent |
| 9        | 1.14    | .69     | .42     | 1.56    | .03     | .45     |
| 10       | 1.18    | .74     | .45     | 1.46    | 1.10    | 1.55    |
| 11       | 1.15    | .65     | .42     | 1.52    | 1.64    | 2.06    |

Specimens of these heats of 1¼" diameter turned to 1" diameter by 3" in length were normalized at 1600° F. and water quenched from about 1475° F. The room temperature Rockwell C hardness in the as quenched and after drawing at 550° F. for 28 hours is given in the following Table V:

TABLE V

| Heat No. | As-Quenched         | Drawn, 550° F.<br>for 28 Hrs. | Difference |
|----------|---------------------|-------------------------------|------------|
| 9        | R <sub>c</sub> 67.2 | R <sub>c</sub> 58.2           | 9.0        |
| 10       | R <sub>c</sub> 66.5 | R <sub>c</sub> 62.0           | 4.5        |
| 11       | R <sub>c</sub> 61.4 | R <sub>c</sub> 58.4           | 3.0        |

This table shows that the steel containing less than 1% aluminum plus silicon and the steel

45 This clearly shows that a total aluminum plus silicon of over 1.75% results in the steel not only having poor hardenability but also are not satisfactory for hot working by commercial mill practices.

50 This is a continuation of my copending application Serial No. 109,803, filed August 11, 1949, now abandoned.

55 While I have shown and described several specific embodiments of my invention, it will be understood that these embodiments are merely for the purpose of illustration and description and that various other forms may be devised within the scope of my invention, as defined in the appended claims.

60 I claim:

65 1. A bearing steel characterized by good forgeability and by high hardenability and retention of hardness after quenching from above its  $A_{e1}$  point and thereafter subjected to prolonged heating at 550° F., said steel containing from about .95 to 1.15% carbon, .25 to .60% manganese, .35% maximum nickel, 1.35 to 1.65% chromium, .35% maximum copper, .75 to 1.25% aluminum and .20 to .50% silicon, the total of 70 aluminum plus silicon being between about 1.00 and 1.75%, the balance being iron and residual amounts of other elements.

75 2. A bearing steel characterized by good forgeability and by a hardness in excess of 60 R<sub>c</sub> after water quenching from about 1475° F. re-

tention of room temperature hardness in excess of 60 R<sub>c</sub> after prolonged heating at 550° F., said steel containing from about .95 to 1.15% carbon, .25 to .60% manganese, .35% maximum nickel, 1.35 to 1.65% chromium, .35% maximum copper, .75 to 1.25% aluminum and .20 to .50% silicon, the total of aluminum plus silicon being between about 1.00 and 1.75, the balance iron and residual amounts of other elements.

KARL F. SCHAUWECKER.

## References Cited in the file of this patent

## FOREIGN PATENTS

| 5 | Number  | Country | Date          |
|---|---------|---------|---------------|
|   | 658,823 | Germany | Apr. 14, 1938 |